

3,184,373

**FILLED PAPER CONTAINING A MIXTURE OF RESIN AND MUCILAGINOUS MATERIAL AS A RETENTION AID AND PROCESS FOR PRODUCING SAID PAPER**

Hanns F. Arledter, Chillicothe, Ohio, assignor, by mesne assignments, to The Mead Corporation, a corporation of Ohio

No Drawing. Continuation of application Ser. No. 600,410, July 27, 1956. This application July 5, 1961, Ser. No. 121,827

The portion of the term of the patent subsequent to

June 28, 1977, has been disclaimed

14 Claims. (Cl. 162—152)

This application is a continuation of my copending application Serial No. 600,410, filed July 27, 1956, now abandoned.

The present invention relates to paper and a process for producing the same, and more particularly to a high filler content paper and a process for producing the same.

Water-laid papers have been prepared heretofore having a relatively high filler content but having a filler retention in the range from about 50% to about 70% only. This low filler retention has constituted a serious drawback to the production of such papers, since from about 50% to about 30% of the filler particles originally added to the paper stock have passed through the wire of the papermaking machine without being retained in the paper and accordingly have been lost in the white water.

It is, therefore, the principal object of the present invention to provide a water-laid paper having not only high filler content but also a filler retention in excess of about 85% with only insignificant loss of filler particles in the white water, and a process of producing such a paper. Additional objects are to provide a paper having no two-sidedness, good dewatering rate, and very little dusting.

The product of the present invention is a paper consisting of a water-laid interfelted fibrous web containing fibers, filler particles, and a synergistic mixture of filler retention aids. The synergistic mixture of filler retention aids makes possible the production of a paper having a remarkable filler particle retention in excess of about 85%, and as high as about 99%, even in papers having a high filler content.

The paper contains from about 20% to about 90% of any fibers of papermaker length, i.e., less than 6 millimeters, or longer, e.g., 6-15 millimeters. The fibers which can be employed either alone or in admixtures include, for example, the following: so-called "papermaking fibers," such as kraft, alpha-cellulose, sulfite cellulose, cotton, hemp, rag, esparto, straw, bagasse, and the like; synthetic organic fibers such as those formed from polyamide resins made by the polymerization of a hexamethylene diamine salt of adipic acid (Nylon), polytetrafluoroethylene fibers (Teflon), synthetic fibers made by the condensation of dimethyl terephthalate and ethylene glycol (Dacron), synthetic fibers made from polyacrylonitrile (Orlon), synthetic fibers made by the copolymerization of 40% acrylonitrile and 60% vinyl chloride (Dynel), polyvinyl chloride fibers, polyvinylidene chloride fibers (Saran), dinitrile fibers, cellulose acetate fibers, cellulose triacetate fibers, and viscose rayon fibers; synthetic inorganic fibers; such as glass, silica, aluminum silicate, steel wool, and the like; and natural inorganic fibers, such as asbestos.

The paper also contains from about 80% to about 10%, respectively, of filler particles, although amounts less than 10% may be employed, if desired. These filler particles preferably have a size in the range from about 60 mesh to about 2,000 mesh. While paper may also

be made in accordance with the invention containing larger size filler particles, such paper has poor uniformity.

The filler particles may be of any nature usable in a paper and include solid particles as well as liquid particles. The liquid particles, such as those present in emulsions and latices, may serve as binders for the paper. The filler particles may be, for example, the conventional fillers used in the manufacture of paper, such as zinc sulfide, titanium dioxide, clay, talc, diatomaceous earth, barium sulfate, alumina, and other water-insoluble inorganic compounds. The filler particles may also be metallic powders or flitters, such as silver, aluminum, gold, lead, tantalum, nickel, iron, and copper. Any water-insoluble thermoplastic or thermosetting resin which can be manufactured in powder form may be used in the paper to supply the filler particle content. The following thermosetting resin powders are typical of those which can be employed either alone or in mixture; phenolic resins, such as phenol-formaldehyde resins or phenol furfural resins; benzoguanamine formaldehyde resins; diallylphthalate polymers; and silicone resins. Suitable thermoplastic resin powders include, for example, polyacrylic resins, such as polymethylmethacrylate; polyvinyl chloride; cellulose acetate; cellulose butyrate; poly-

styrene; polyethylene; polyvinyl butyral; polytetrafluoroethylene (Teflon); and polyvinyl acetate. Suitable fillers also include wood dust, pigments, and fluorescent or luminescent materials. Other suitable fillers include flocculated particles of so-called beater addition resins, latices, etc., of the nature of neoprene latex (polychloroprene), rubber latex, acrylic resin emulsions (Rhoplex WN), polyvinyl acetate emulsions (117-SS), polystyrene latices, and phenol-formaldehyde resin dispersions which may serve as binders for the paper.

In addition to the fibers and filler particles, the paper contains a synergistic mixture of filler retention aids. The first component of the synergistic mixture is a water-soluble mucilaginous material, such as guar gum, methylated guar gum, mannogalactan, sodium alginate (Keltex), or protein substances. The paper contains from about 0.1% to about 2% of such materials based on the solids content of the paper. The second component of the synergistic mixture, which is added later in the process, is water-soluble polyethyleneimine resin, sold under the trade names "PEI" or "Polymins P," water-soluble melamine formaldehyde resin, or water-soluble urea melamine resin, or mixtures thereof, from about 0.1% to about 2% of the material being employed based upon the solids content of the paper. An appreciably larger amount of these retention aids is undesirable, since such a larger amount may serve to decrease the filler retention properties thereof or may yield other unwanted effects. This synergistic mixture of retention aids makes possible the preparation of a high filler content paper with filler particle retention in excess of about 85% by the obtention of large flocs of the fibers and filler particles in the paper furnish, so that the filler particles are not lost through the wire of a papermaking machine into the white water.

In the foregoing and in the examples to follow, the retention aids are described as "water-soluble." These materials, as will be recognized by those skilled in the art, are high molecular weight polymers which, even though molecularly dispersed in water, yield solutions having the characteristics of colloidal dispersions in terms of viscosity and presence of the Tyndal effect.

It will be appreciated that water-laid filled papers may be produced having a filler retention in excess of 50% without the use of any filler retention aid. Accordingly, in order to show a synergistic effect by the use of filler retention aids, it is necessary to calculate the synergistic

effect as the excess amount of filler retained above the retention level obtained without the presence of any filler retention aid. The synergistic effect of the mixture of filler retention aids is readily shown by the data presented in the examples below:

## EXAMPLE 1

The following papers were prepared:

## Paper A-1

|                                   |       |            |
|-----------------------------------|-------|------------|
| Alpha-cellulose fibers            | ----- | Percent 10 |
|                                   | 33    | 33         |
| Titanium dioxide filler particles | ----- | 67         |
|                                   | 58.2  | 58.2       |
| Percent material retained on wire | ----- | 15         |

## Paper A-2

|                                                                                     |       |      |      |
|-------------------------------------------------------------------------------------|-------|------|------|
| Alpha-cellulose fibers                                                              | ----- | 33   | 33   |
| Titanium dioxide filler particles                                                   | ----- | 67   | 67   |
| Melamine formaldehyde resin (based on alpha-cellulose and titanium dioxide content) | ----- | 1    | 1    |
| Percent material retained on wire                                                   | ----- | 51   | 20   |
| Net change in filler retention compared with Paper A-1                              | ----- | -7.2 | -7.2 |

## Paper A-3

|                                                                           |       |       |       |
|---------------------------------------------------------------------------|-------|-------|-------|
| Alpha-cellulose fibers                                                    | ----- | 33    | 25    |
| Titanium dioxide filler particles                                         | ----- | 67    | 69    |
| Polyethyleneimine (based on alpha-cellulose and titanium dioxide content) | ----- | 1     | 30    |
| Percent material retained on wire                                         | ----- | 51    | 20    |
| Net change in filler retention compared with Paper A-1                    | ----- | +10.8 | +10.8 |

## Paper A-4

|                                                                  |       |       |       |
|------------------------------------------------------------------|-------|-------|-------|
| Alpha-cellulose fibers                                           | ----- | 33    | 35    |
| Titanium dioxide filler particles                                | ----- | 67    | 35    |
| Guar gum (based on alpha-cellulose and titanium dioxide content) | ----- | 1     | 1     |
| Percent material retained on wire                                | ----- | 72    | 72    |
| Net change in filler retention compared with Paper A-1           | ----- | +13.8 | +13.8 |

## Paper A-5

|                                                                           |       |       |       |
|---------------------------------------------------------------------------|-------|-------|-------|
| Alpha-cellulose fibers                                                    | ----- | 33    | 45    |
| Titanium dioxide filler particles                                         | ----- | 67    | 88    |
| Guar gum (based on alpha-cellulose and titanium dioxide content)          | ----- | 1     | 50    |
| Polyethyleneimine (based on alpha-cellulose and titanium dioxide content) | ----- | 45    | 50    |
| Percent material retained on wire                                         | ----- | 29.8  | +29.8 |
| Net change in filler retention compared with Paper A-1                    | ----- | +29.8 | +29.8 |

## Paper A-6

|                                                                               |       |     |     |
|-------------------------------------------------------------------------------|-------|-----|-----|
| Alpha-cellulose fibers                                                        | ----- | 33  | 33  |
| Titanium dioxide filler particles                                             | ----- | 67  | 70  |
| Guar gum (based on alpha-cellulose and titanium dioxide content)              | ----- | 1   | 1   |
| Melamine formaldehyde (based on alpha-cellulose and titanium dioxide content) | ----- | 0.5 | 0.5 |
| Polyethyleneimine (based on alpha-cellulose and titanium dioxide content)     | ----- | 75  | 75  |

## Paper A-6—Continued

|                                                        |       |       |
|--------------------------------------------------------|-------|-------|
| Percent material retained on wire                      | ----- | 92.5  |
| Net change in filler retention compared with Paper A-1 | ----- | +34.3 |

In comparing Papers A-3, A-4, and A-5 it will be noted that the expected effect of adding 1% water-soluble polyethyleneimine plus 1% water-soluble guar gum, both based on the solids content of the paper, to Paper A-1 would be the sum of +10.8% and +13.8%, or +24.6% increase in filler retention. However, it will be noted that in Paper A-5 the net change in filler retention was +29.8% as compared with the expected change of +24.6%, indicating a clear case of synergism.

## EXAMPLE 2

In this example a series of papers were prepared using the following stock: 77% alpha-cellulose fibers (400 parts), 11.5% zinc sulfide filler particles (60 parts), and 11.5% titanium dioxide filler particles (60 parts). In the following tabulation the amounts of additives are based on the solids content of the paper.

| Paper | Additives                                           | Stock retention, percent | Net change in filler retention compared with paper B-1, percent |
|-------|-----------------------------------------------------|--------------------------|-----------------------------------------------------------------|
| B-1   | None                                                | 75                       | -----                                                           |
| B-2   | 0.2% guar gum                                       | 83                       | +8                                                              |
| B-3   | 0.5% melamine formaldehyde resin                    | 55                       | -20                                                             |
| B-4   | 0.2% guar gum plus 0.5% melamine formaldehyde resin | 91                       | +16                                                             |

In comparing Papers B-2, B-3, and B-4 it will be noted that the expected net change in the addition of water-soluble guar gum plus water-soluble melamine formaldehyde resin to Paper B-1 would be the sum of +8% and -20%, or -12%, while actually in Paper B-4 the net change in filler retention was +16%, clearly indicating a remarkable synergistic effect.

## EXAMPLE 3

In this example the following paper stock was used: 53% alpha-cellulose fibers (225 parts), 23.5% titanium dioxide filler particles (100 parts), and 23.5% diatomaceous earth filler particles (100 parts).

| Paper | Additives                                           | Percent filler found in paper | Filler retention, percent | Net change in filler retention compared with paper C-1, percent |
|-------|-----------------------------------------------------|-------------------------------|---------------------------|-----------------------------------------------------------------|
| C-1   | None                                                | 39.5                          | 82                        | -----                                                           |
| C-2   | 0.4% melamine formaldehyde resin                    | 37.2                          | 79                        | -3                                                              |
| C-3   | 0.2% guar gum                                       | 41.9                          | 89                        | +7                                                              |
| C-4   | 0.2% guar gum plus 0.4% melamine formaldehyde resin | 45.4                          | 96.5                      | +14.5                                                           |

In the above table the amount of water-soluble melamine formaldehyde resin and water-soluble guar gum additives is based upon the total solids content of the paper. In comparing Papers C-2, C-3, and C-4 it will be noted that the combination of melamine formaldehyde resin and guar gum would be expected to produce a net change in filler retention compared with Paper C-1 of -3% plus +7%, or +4%, while actually the combination of guar gum and melamine formaldehyde resin as

shown in Paper C-4 produced a net change in filler retention of +14.5%, clearly indicating a remarkable synergistic effect once again.

## EXAMPLE 4

The fiber and filler losses in the manufacture of a paper can be determined from the white water losses as shown by this example. In the example the following paper furnish was used: 33% sulfite cellulose fibers (450 grams), 67% clay filler particles (900 grams), 200 liters water, and sufficient alum to pH 4.6.

| Paper  | Additives                                                                                           | Stock retention, percent | Net change in retention compared with paper F-1, percent |
|--------|-----------------------------------------------------------------------------------------------------|--------------------------|----------------------------------------------------------|
|        |                                                                                                     |                          |                                                          |
| 5 F-1  | None                                                                                                | 78                       |                                                          |
| 5 F-2  | 0.5% melamine formaldehyde resin                                                                    | 77                       | -1                                                       |
| 10 F-3 | 0.2% guar gum                                                                                       | 79.5                     | +1.5                                                     |
| 10 F-4 | 0.5% melamine formaldehyde resin plus 0.2% guar gum                                                 | 85                       | +7                                                       |
| 10 F-5 | 0.5% melamine formaldehyde resin plus 0.2% guar gum plus 0.5% polyethyleneimine (ammonia to pH 7.0) | 89                       | +11                                                      |

| Paper | Additives                                           | White water losses in grams per liter | Stock retention, percent | Net change in retention compared with paper D-1, percent |
|-------|-----------------------------------------------------|---------------------------------------|--------------------------|----------------------------------------------------------|
| D-1   | None                                                | 1.98                                  | 70                       |                                                          |
| D-2   | 0.5% melamine formaldehyde resin                    | 2.22                                  | 67                       | -3                                                       |
| D-3   | 0.5% guar gum                                       | 0.89                                  | 86.8                     | +16.8                                                    |
| D-4   | 0.5% guar gum plus 0.5% melamine formaldehyde resin | 0.37                                  | 94.5                     | +24.5                                                    |

In the above table the amount of water-soluble melamine formaldehyde resin as well as the amount of water-soluble guar gum is based upon the solids content of the paper. In comparing Papers D-2, D-3, and D-4 it will be seen that the addition of both guar gum and melamine formaldehyde resins to the paper stock would be expected to produce a net change in retention of -3% plus +16.8%, or +13.8%, while in actuality as shown by Paper D-4 the net change in retention was considerably greater than this amount, and in particular +24.5%.

Under equal conditions a stock retention of 93.6% was obtained when zinc sulfide filler particles were used in lieu of the clay filler particles. Also, when 75% diatomaceous earth filler particles were substituted for the clay filler particles, a stock retention of approximately 94.5% was obtained by the use of the synergistic mixture of retention aids, i.e., water-soluble guar gum plus water-soluble melamine formaldehyde resin or water-soluble polyethyleneimine resin.

## EXAMPLE 5

Papers were prepared from the following paper furnish and tested for stock retention: 33% of glass fibers (33 parts), 67% of 100 mesh water-insoluble Vinylite powder (copolymer of vinyl chloride and vinyl acetate) (67 parts), and 10,000 parts of water. In the following tabulation the amounts of additives are based upon the solids content of the paper.

| Paper | Additives                    | Stock retention, percent | Net change in retention compared with paper E-1, percent |
|-------|------------------------------|--------------------------|----------------------------------------------------------|
| E-1   | None                         | 82                       |                                                          |
| E-2   | 0.2% guar gum                | 88                       | +6                                                       |
| E-3   | 0.5% PEI (polyethyleneimine) | 86.5                     | +4.5                                                     |
| E-4   | 0.2% guar gum plus 0.5% PEI  | 93.5                     | +11.5                                                    |

Once again synergism has been shown in the comparison on Papers E-2, E-3, and E-4. When water-soluble guar gum plus water-soluble polyethyleneimine are used in combination, it would be expected that the net change in retention would amount to the sum of +6% plus +4.5%, or +10.5%, while actually a net change in retention of +11.5% was obtained in Paper E-4.

## EXAMPLE 6

Papers were formed from the following paper furnish: 50% water-insoluble phenol formaldehyde resin powder, 50% alpha-cellulose fibers, and alum to pH 4.8.

Without flocculation by use of the filler retention aids, the retention is between 45% and 55%.

## EXAMPLE 8

The following paper stock was formed into a paper and the percent filler retention noted as influenced by the temperature of flocculation: 67% zinc sulfide filler particles, 33% alpha-cellulose fibers, and 10,000 parts water. In the tabulation below the amount of additives is based on the solids content of the paper.

| Paper | Additives                                           | Percent retained on wire |         | Net change in retention compared with paper H-1, percent |         |
|-------|-----------------------------------------------------|--------------------------|---------|----------------------------------------------------------|---------|
|       |                                                     | 68° F.                   | 130° F. | 68° F.                                                   | 130° F. |
| H-1   | None                                                | 53                       | 56      |                                                          |         |
| H-2   | 0.5% melamine formaldehyde resin                    | 49                       | 46.6    | -4                                                       | -9.4    |
| H-3   | 0.5% guar gum                                       | 61                       | 67      | +8                                                       | +11     |
| H-4   | 0.5% melamine formaldehyde resin plus 0.5% guar gum | 72                       | 82      | +19                                                      | +14     |
| H-5   | 0.5% polyethyleneimine                              |                          |         |                                                          |         |
| H-6   | 0.5% guar gum plus 0.5% polyethyleneimine           |                          |         |                                                          |         |
|       |                                                     | 72.2                     |         |                                                          | +16.2   |
|       |                                                     | 86                       |         |                                                          | +30     |

## EXAMPLE 9

In this example a series of papers were prepared using the following stock having liquid filler particles: 50 grams of alpha-cellulose fibers, 100 grams of neoprene latex (36% neoprene content), and 10 gallons of water. In the following tabulation, the amounts of additives are based on the solids content of the paper.

| Paper | Additives                                                                   | Stock retention, percent |
|-------|-----------------------------------------------------------------------------|--------------------------|
| J-1   | Alum to pH 6.4                                                              | 56                       |
| J-2   | 0.5% guar gum                                                               | 53                       |
| J-3   | 1% polyethyleneimine                                                        | 60                       |
| J-4   | 3% polyethyleneimine                                                        | 76                       |
| J-5   | 1% melamine formaldehyde resin                                              | 53                       |
| J-6   | 0.5% guar gum plus 1% melamine formaldehyde resin plus 1% polyethyleneimine | 92.5                     |

The paper having high filler content and high filler retention may be prepared by any process which does not destroy the flocs produced by the synergistic filler retention aids. Accordingly, the paper may be prepared by any process wherein the flocculated fibers and fillers are not subjected to violent mechanical action. If the flocs are formed in the mixing chamber of the headbox, they are not subjected to violent mechanical action as would be the case if the flocs were exposed to the action of the beater roll, fan pump, high speed agitator in the beater or machine chest, or the action of the vibrating screen ahead of the headbox. If the flocs are subjected to violent mechanical action, the effect of the synergistic mixture of filler retention aid is inhibited, so that there is no longer obtained high filler retention and sheet uniformity.

The paper may, therefore, be prepared by pumping an aqueous slurry of the fibers, filler particles and water-soluble mucilaginous material to the mixing chamber of the headbox of a papermaking machine, adding thereto the water-soluble polyethyleneimine, melamine formaldehyde, or urea melamine resins, or mixtures thereof, to flocculate the fibers and filler particles with minimum agitation, forming the paper web on the wire of the papermaking machine, and dewatering, drying, and calendering the web. The flocculation of the filler particles and fibers is preferably conducted at a pH in the range from about 6 to about 7 and at a temperature above room temperature, preferably in the range from about 90° F. to about 140° F., in order to obtain maximum filler retention.

The preferred embodiment of the process of the invention comprises pumping an aqueous slurry heated to 120° F. of about one-tenth of the fibrous content of the paper along with all of the filler particles and water-soluble mucilaginous material to the mixing chamber of the headbox of a papermaking machine, adding thereto water-soluble polyethyleneimine, melamine formaldehyde, or urea melamine resins, or mixtures thereof to flocculate the fibers and filler particles at elevated temperature, mixing the flocculated heated slurry with an aqueous unheated slurry of nine-tenths of the fibrous content of the paper with minimum agitation to flocculate the added fibers, forming a paper web on the wire of the paper-

making machine, and dewatering, drying, and calendering the web. Whether the flocculated slurry is added to the fiber slurry, or vice versa, is immaterial. This preferred process permits the production of paper having maximum filler content and filler retention.

The process of the invention may be further improved by re-employing the white water. The filler content and filler retention of the paper may also be further improved by adding sufficient sodium abietate of a pH of 11.0 to the fiber-filler slurry containing the synergistic mixture of retention aids and then adding thereto sufficient papermaker's alum to lower the pH to from about 4.5 to about 4.8.

The high filler content paper having high filler retention has been illustrated by the examples set forth above. The paper of the invention as well as the process of the invention will be further illustrated by the examples presented below.

## EXAMPLE 10

500 parts of kraft paper was beaten in a beater to a beating degree of 17° S.R. at a stock consistency of 6%. The stock was brought over beater chest, refiner, machine chest, screen and vortrap to the mixing chamber of the headbox of a paper machine. The stock was here diluted, in the conventional manner with the white water from the tray of the paper machine to a stock consistency of 5 grams per liter and formed Stock A containing in all 100,000 parts of water.

50 parts of kraft pulp in 1,000 parts of water was beaten separately to a beating degree of 28° S.R. and mixed in a mixing chamber before the headbox with 500 parts of powdered water-insoluble phenol formaldehyde resin of a size of 200 mesh plus 1,000 parts of water. To the resin-fiber slurry there was added 4 parts of dissolved guar gum. The fiber plus resin powder slurry containing the water-soluble guar gum was then diluted with water to 10,000 parts of liquid and flocculated with 3 parts of water-soluble melamine formaldehyde resin dissolved in 100 parts of water. This formed Stock B.

Stock A and Stock B were then gently mixed together with minimum agitation in the mixing chamber of the headbox of a paper machine for approximately 5 seconds to flocculate the fibers in Stock A and fed to the wire of the papermaking machine, dewatered, dried, and calendered into a paper.

The paper product contained 53% of kraft fibers, 47% of phenol formaldehyde resin powder, 0.4% of water-soluble guar gum based on the solids content of the paper, and 0.3% of water-soluble melamine formaldehyde resin based on the solids content of the paper.

## EXAMPLE 11

50 parts of sulfite cellulose of a beating degree of 42° S.R. in 10,000 parts of water was mixed with 200 parts of zinc sulfide powder and 800 parts of finely ground diatomaceous earth in a mixing chamber before the headbox. 6 parts of water-soluble guar gum, dissolved in 400 parts of water, was added to this paper stock. The stock was diluted to the ratio of 1:10 with water and 5 parts of water-soluble polyethyleneimine added thereto to flocculate the filler and fiber content. This stock formed Stock A.

450 parts of sulfite cellulose was beaten to a beating degree of 27° S.R. at a stock consistency of 6% and diluted in the machine chest to 3% stock consistency. This formed Stock B. Stock B was diluted with white water to a stock consistency of 5 grams per liter and pumped to the mixing chamber of the headbox of a paper machine at a rate of 30 parts of sulfite cellulose per minute.

Stock A was added to Stock B (30 parts) at a rate of 60 parts dry material per minute and gently mixed together with minimum agitation. The stock was then fed upon the wire of the papermaking machine, dewatered, dried, and calendered.

The paper product so formed had excellent printability and contained 33% sulfite cellulose, 67% filler particles (zinc sulfide plus diatomaceous earth), 0.4% water-soluble guar gum based on the solids content of the paper, and 0.3% water-soluble polyethyleneimine based on the solids content of the paper.

#### EXAMPLE 12

50 parts of glass fibers having a diameter of 1.5 microns in 20,000 parts of water was mixed with 600 parts of water-insoluble diallylphthalate resin powder in a mixing chamber before the headbox. 3 parts of water-soluble guar gum was then added thereto and the slurry flocculated with 5 parts of water-soluble urea melamine resin, thereby forming Stock A.

400 parts of glass fibers having a diameter of 3 microns was beaten, diluted with white water, and pumped to the mixing chamber of the headbox of a paper machine to form Stock B.

Stock A was added to Stock B, gently mixed together with minimum agitation, and a paper product formed by feeding the resultant flocculated slurry to the wire of the papermaking machine, dewatering, drying, and calendering the web so produced.

The paper product contained 44% glass fibers, 56% diallylphthalate resin powder filler, 0.3% water-soluble guar gum based on the solids content of the paper, and 0.5% water-soluble urea melamine resin based on the solids content of the paper. The paper product had a resin retention of 97%.

#### EXAMPLE 13

500 pounds of kraft pulp was beaten in a beater to a beating degree of 17° S.R. at a stock consistency of 6%. 500 pounds of water-insoluble phenol formaldehyde resin powder with a softening point of 70° C.-85° C. and a screen mesh size ranging from 80 to 200 was dispersed in 5,000 pounds of water containing 0.5 pound of high viscosity methyl cellulose. The beaten kraft pulp and the phenol formaldehyde resin powder suspension was then mixed in the machine chest. The stock consistency was lowered to 2.45% and 5 pounds of cold water-soluble guar gum added thereto. The stock was pumped to the mixing chamber of the headbox of a paper machine and flocculated at around 2.35% stock consistency, pH 7.0, with a 2.5% solution containing 6 pounds of water-soluble urea melamine resin. The stock consistency was then reduced to 1.0% with white water and aluminum sulfate (alum) added to obtain a pH of 4.5. Shortly before the stock went on the wire of the paper machine a solution of 0.5% sodium abietate of pH 11 was added in such an amount that approximately 1.8% resin was added to the stock. The flocculated fiber-filler slurry was then fed to the wire of the papermaking machine, dewatered, dried, and calendered into a paper product containing 50% kraft fibers, 50% phenol formaldehyde resin powder, 0.5% water-soluble guar gum based on the solids content of the paper, and 0.6% water-soluble urea melamine resin based on the solids content of the paper.

#### EXAMPLE 14

25 parts of glass fibers of 3 micron diameter, 12.5 parts of viscose rayon fibers, 12.5 parts of cellulose fibers, and 100 parts of polyvinyl acetate emulsion of 50% resin content was mixed in 10,000 parts of water. Alum was added to a pH of 5.0, ammonia added to a pH of 9.0, and the pH finally adjusted to 7.0 with alum to flocculate the slurry. The flocculated stock mixture was pumped to the headbox of a Fourdrinier machine and 0.5% water-soluble guar gum and 1% of a water-soluble polyethyleneimine and water-soluble melamine formaldehyde mixture added. A paper product was then formed in the conventional manner.

The paper product contained 25% glass fibers, 50% polyvinyl acetate, 12.5% viscose rayon fibers, and 12.5%

cellulose fibers, as well as 0.5% water-soluble guar gum and 1% water-soluble polyethyleneimine plus water-soluble melamine formaldehyde resin based on the solids content of the paper. The product had a resin retention of 94%.

Data showing synergism are presented below.

|    |                                                                                            | Stock retention,<br>percent |
|----|--------------------------------------------------------------------------------------------|-----------------------------|
|    | Additives:                                                                                 |                             |
| 10 | Alum added to pH 5.0                                                                       | 48                          |
|    | Alum added to pH 5.0, ammonia to pH 8.8                                                    | 66                          |
|    | Alum added to pH 5.0, ammonia to pH 9.0, and alum to pH 7.0                                | 78                          |
| 15 | 0.5% guar gum                                                                              | 52                          |
|    | 1% polyethyleneimine                                                                       | 56                          |
|    | Alum to pH 5.0, ammonia to pH 9.0, alum to pH 7.0, 0.5% guar gum, and 1% polyethyleneimine | 96                          |

#### EXAMPLE 15

9 part of viscose rayon fibers (5.5 denier, 6 mm. length), 1 part of viscose rayon fibers (0.75 denier, 4 mm. length), and 20 parts of neoprene emulsion (36%) were dispersed in 6,000 parts water of a pH of 5.2. Ammonia was added to a pH of 9.2. Alum was added to a pH of 6.4 and the slurry then flocculated in the headbox with 1% water-soluble guar gum and 1% water-soluble polyethyleneimine. A well-bonded strong paper, containing approximately 6% binder, was obtained.

The high filler content paper of the invention may be used for decorative laminates, flame retardant laminates, chemical resistant laminates, and also for printing papers and the production of films by exposing the paper to heat and pressure in a calender.

Various modifications and changes may be made in the invention herein set forth without departing from the spirit thereof and accordingly the invention is to be limited only within the scope of the appended claims.

I claim:

1. A filled paper having a filler retention in excess of about 85% consisting of a water-laid interfelted fibrous web consisting of from about 10% to about 80% of filler particles, from about 90% to about 20% respectively of fibers, and a synergistic filler retention mixture of from about 0.1% to about 2% of a water-soluble mucilaginous material selected from the group consisting of mannogalactan and sodium alginate based on the solids content of the paper, and from about 0.1% to about 2% of at least one water-soluble resin selected from the group consisting of polyethyleneimine, melamine formaldehyde, and urea melamine resins based on the solids content of the paper.
2. A paper as set forth in claim 1 wherein the filler particles are water-insoluble resin powder.
3. A paper as set forth in claim 1 wherein the filler particles are water-insoluble inorganic compounds.
4. A paper as set forth in claim 1 wherein the filler particles are flocculated liquid particles.
5. A paper as set forth in claim 1 wherein the fibers are cellulosic fibers.
6. A paper as set forth in claim 1 wherein the fibers are synthetic organic fibers.
7. A paper as set forth in claim 1 wherein the fibers are synthetic inorganic fibers.
8. A paper as set forth in claim 1 wherein the fibers are natural inorganic fibers.
9. The process of preparing a filled paper having a filler retention in excess of about 85% comprising pumping an aqueous slurry consisting of water, from about 20% to about 90% of fibers, from about 80% to about 10% respectively of filler particles, and from about 0.1% to about 2% of a water-soluble mucilaginous material selected from the group consisting of a mannogalactan and sodium alginate based on the solids content of the paper to the headbox of a papermaking machine; adding from about 0.1% to about 2% based on the solids content of the paper of at least one water-soluble resin selected from

the group consisting of polyethyleneimine, melamine formaldehyde, and urea melamine resins thereto with minimum agitation to form a synergistic filler retention mixture and to flocculate the fibers and filler particles; forming a paper web on the wire of the papermaking machine; and dewatering, drying, and calendering the web.

10. The process as set forth in claim 9 wherein the flocculation is conducted at a pH in the range from about 6 to about 7.

11. The process as set forth in claim 9 wherein the flocculation is conducted at a temperature in the range from about 90° F. to about 140° F.

12. The process as set forth in claim 9 wherein after the addition of the resin there is added alkaline sodium abietate to adjust the pH of the flocculated slurry to about 8.5 and then there is added alum to further adjust the pH of the flocculated slurry to about 4.6-4.8.

13. The process of preparing a filled paper having a filler retention in excess of about 85% comprising mixing a flocculated aqueous slurry consisting of water, about one-tenth of the 90-20% fibrous content of the paper, from about 10% to about 80% respectively of filler particles, and a synergistic filler retention mixture of from about 0.1% to about 2% based on the weight of the 25 solids content of the paper of a water-soluble mucilaginous material selected from the group consisting of a mannosgalactan and sodium alginate and from about 0.1% to about 2% based on the solids content of the paper of at least one water-soluble resin selected from the group consisting of polyethyleneimine, melamine formaldehyde and urea melamine resins with an aqueous slurry con-

5

10

sisting of water and nine-tenths of the 90-20% fibrous content of the paper in the headbox of a papermaking machine with minimum agitation; forming a paper web on the wire of the papermaking machine; and dewatering, drying, and calendering the web.

14. The process as set forth in claim 13 wherein the aqueous slurry of about one-tenth of the fibrous content of the paper has a temperature in the range of from about 90° F. to about 140° F. and the slurry containing nine-tenths of the fibrous content of the paper is unheated.

## References Cited by the Examiner

## UNITED STATES PATENTS

|           |       |                |         |
|-----------|-------|----------------|---------|
| 2,071,025 | 2/36  | Colbert et al. | 162-168 |
| 2,336,797 | 12/43 | Maxwell        | 162-157 |
| 2,366,400 | 1/45  | Harrison       | 162-166 |
| 2,378,193 | 6/45  | Cummins        | 162-166 |
| 2,526,125 | 10/50 | Francis        | 162-140 |
| 2,563,897 | 8/51  | Wilson et al.  | 162-166 |
| 2,680,682 | 6/54  | Dearing        | 162-168 |
| 2,685,508 | 8/54  | Spear          | 162-178 |
| 2,687,447 | 8/54  | Merrill        | 162-166 |
| 2,694,630 | 11/54 | Landes et al.  | 162-166 |
| 2,698,793 | 1/55  | Landes et al.  | 162-164 |
| 2,773,763 | 12/56 | Scott          | 162-145 |
| 2,786,759 | 3/57  | Feigley        | 162-168 |
| 2,943,013 | 6/60  | Arledter       | 162-166 |
| 3,052,595 | 9/62  | Pye            | 162-181 |

DONALL H. SYLVESTER, Primary Examiner.

RICHARD D. NEVIUS, MORRIS O. WOLK, Examiners.